



US007884143B2

(12) **United States Patent**  
**Fournier et al.**

(10) **Patent No.:** **US 7,884,143 B2**  
(45) **Date of Patent:** **Feb. 8, 2011**

(54) **BIOPOLYMER-BASED COMPOSITION FOR  
A POWER AND/OR  
TELECOMMUNICATIONS CABLE**

2003/0162040 A1 8/2003 Matsumoto

(75) Inventors: **Jérôme Fournier**, Lyons (FR); **Sophie Barbeau**, Genas (FR)

FOREIGN PATENT DOCUMENTS

(73) Assignee: **Nexans**, Paris (FR)

|    |              |           |
|----|--------------|-----------|
| DE | 19632504     | 2/1998    |
| EP | 0714914      | 6/1996    |
| EP | 0784994      | 7/1997    |
| GB | 515666       | 12/1939   |
| GB | 588210       | 5/1947    |
| JP | 2004-4311063 | * 11/2004 |
| JP | 2004311063   | 11/2004   |

(\*) Notice: Subject to any disclaimer, the term of this patent is extended or adjusted under 35 U.S.C. 154(b) by 453 days.

(21) Appl. No.: **12/005,133**

OTHER PUBLICATIONS

(22) Filed: **Dec. 21, 2007**

French International Search Report—Aug. 9, 2007.  
International Search Report dated May 27, 2008.

(65) **Prior Publication Data**

\* cited by examiner

US 2008/0153941 A1 Jun. 26, 2008

*Primary Examiner*—Robert D. Harlan

(30) **Foreign Application Priority Data**

(74) *Attorney, Agent, or Firm*—Sofer & Haroun, LLP

Dec. 26, 2006 (FR) ..... 06 55944

**ABSTRACT**

(51) **Int. Cl.**  
**C09K 3/00** (2006.01)

The present invention relates to a power and/or telecommunications cable including at least one component element made of a material extruded from an extrudable composition, wherein said extrudable composition comprises a biopolymer selected from polymers of cellulose ester, polymers of starch complexed with a biodegradable polyester, polymers of poly-hydroxyalkanoate, and/or polymers of polylactic acid comprising a mixture of polylactic and of polyester.

(52) **U.S. Cl.** ..... **523/173**

(58) **Field of Classification Search** ..... 523/173  
See application file for complete search history.

(56) **References Cited**

**10 Claims, No Drawings**

U.S. PATENT DOCUMENTS

2,549,101 A 4/1951 Koch ..... 117/128.4  
5,847,031 A 12/1998 Klimmek et al. ..... 524/44



and about 60% by weight polyester, or comprising about 10% by weight polylactic acid and about 90% by weight polyester.

In a particular embodiment, the extrudable composition further includes a fire-retardant filler.

Preferably, the fire-retardant filler is selected from aluminum trihydroxide  $\text{Al}(\text{OH})_3$ , magnesium dihydroxide  $\text{Mg}(\text{OH})_2$ , a mixture of hydrated magnesium carbonate and calcium and magnesium carbonate, zinc borate, and/or caulk powder.

#### MORE DETAILED DESCRIPTION

Other characteristics and advantages of the present invention appear in the light of the examples below, said examples being given by way of non-limiting illustration.

In order to show the advantages obtained with the extrudable compositions of the present invention, Table 1 gives details concerning various samples in accordance with the invention and in accordance with the prior art, for which mechanical and fire-retardant properties have been studied.

The compositions referenced 1 to 5 correspond to a composition of the present invention comprising a biopolymer optionally combined with a synthetic polymer.

The compositions 6 and 7 are compositions forming part of the prior art.

It should be observed that the quantities given in Table 1 are expressed in parts per hundred (pph) parts by weight of polymer.

TABLE 1

| Composition | Ingredients                       |
|-------------|-----------------------------------|
| 1           | 100 pph cellulose                 |
| 2           | 100 pph NF03A starch              |
| 2bis        | 100 pph NF08 starch               |
| 3           | 25 pph NF03A starch and 75 pph PE |
| 4           | 100 pph PHB                       |
| 5           | 100 pph PLA-polyester 467F        |
| 5bis        | 100 pph PLA-polyester 219F        |
| 6           | 100 pph EVA                       |
| 7           | 100 pph PE                        |

The origins of the various ingredients in Table 1 are as follows:

“cellulose” corresponds to the cellulose butyrate acetate polymer referenced Tenite 485E2R30010 sold by the supplier Eastman;

“NF03A starch” corresponds to the starch polymer complex with a biodegradable polyester, referenced Mater-bi NF031 and sold by the supplier Novamont;

“NF08 starch” corresponds to the starch polymer complex with a biodegradable polyester referenced Mater-bi NF08 and sold by the supplier Novamont;

“PHB” corresponds to the polyhydroxide butyrate polymer referenced P209 and sold by the supplier Biomer;

“PLA-polyester 467F” corresponds to the polylactic acid polymer referenced 467F comprising about 40% by weight polylactic acid and about 60% by weight polyester, and sold by the supplier FKUR;

“PLA-polyester 219F” corresponds to the polylactic acid polymer referenced 219F, comprising about 10% polylactic acid and about 90% polyester, and sold by the supplier FKUR;

“EVA” corresponds to the ethylene vinyl acetate copolymer (a synthetic polymer) referenced EVATANE 2803 and sold by the supplier Arkema; and

“PE” corresponds to the polyethylene (a synthetic polymer) referenced LL4004 and sold by the supplier Exxon.

In order to study mechanical properties, samples 1 to 7 corresponding respectively to the compositions 1 to 7 were prepared using the following protocol:

processing the polymer(s) in an internal mixer; and  
5 molding the composition to form plates in a hot press under a pressure of 100 bar for a period of 5 minutes (min).

After cooling and unmolding, the plates were cut up to provide the samples on which the mechanical tests were carried out.

10 Table 2 summarizes the results of certain measurements made on samples 1 to 7 in order to evaluate their tensile strength and their elongation at break.

TABLE 2

| Sample | Tensile strength (MPa) | Elongation at break (%) |
|--------|------------------------|-------------------------|
| 1      | 33                     | 26                      |
| 2      | 11                     | 500                     |
| 2bis   | 15                     | 240                     |
| 3      | 14                     | 640                     |
| 4      | 17                     | 9                       |
| 5      | 26                     | 410                     |
| 5bis   | 13                     | 430                     |
| 6      | 29                     | 767                     |
| 7      | 16                     | 630                     |

Cone calorimeter analyses were also performed in order to evaluate and compare the fire behavior of the various samples.

This type of analysis, consisting in burning samples in ambient air while subjecting them to external energy radiation at a power density of less than 100 kilowatts per square meter ( $\text{kW/m}^2$ ) and imposed by temperature-controlled radiant heating, serves to obtain the effective heat of combustion expressed in megajoules per kilogram (MJ/kg) and the heat release peak expressed in  $\text{kW/m}^2$ .

For this purpose, each sample was shaped into square plates with a side of 10 centimeters (cm) and a thickness of 3 millimeters (mm).

40 The samples shaped in that way were tested using a cone calorimeter in compliance with the standard ISO 5660-1 relating to heat release from building materials.

The smaller the numerical values of the heat release peak and the effective heat of combustion, the better the fire-proofing properties of the composition.

45 Table 3 summarizes the data collected by the cone calorimetry analyses using the samples of Table 2.

TABLE 3

| Sample | Heat of combustion (MJ/kg) | Heat release peak ( $\text{kW/m}^2$ ) |
|--------|----------------------------|---------------------------------------|
| 1      | 23                         | 910                                   |
| 2      | 21                         | 1030                                  |
| 2bis   | 19                         | 756                                   |
| 4      | 23                         | 755                                   |
| 5      | 22                         | 860                                   |
| 5bis   | 23                         | 228                                   |
| 6      | 37                         | 1360                                  |
| 7      | 43                         | 1310                                  |

50 From the results of Tables 2 and 3, it can clearly be seen that the samples based on biopolymers in accordance with the present invention present mechanical properties and fire resistance properties that are as good as, or even better than, those of prior art polymers PE and EVA.

55 To improve fire resistance properties, new samples including a fire-retardant filler are specified in Table 4.

## 5

Sample 8 is a composition comprising a biopolymer (cellulose), a synthetic polymer (EVA), and magnesium hydroxide.

Samples 9 to 11 correspond respectively to samples 2, 6, and 7 having a fire-retardant filler added thereto.

Samples 12 to 14 correspond to sample 2 having a fire-retardant filler added thereto.

Samples 15 to 17 correspond to sample 5b is having a fire-retardant filler added thereto.

Sample 18 corresponds to sample 2bis having a fire-retardant filler added thereto.

In this respect, it should be observed that the quantities mentioned in Table 4 are expressed in parts per 100 parts of polymer (pph).

TABLE 4

| Sample | Ingredients                                                                                                  | Heat of combustion (MJ/kg) | Heat release peak (kw/m <sup>2</sup> ) |
|--------|--------------------------------------------------------------------------------------------------------------|----------------------------|----------------------------------------|
| 8      | 25 pph cellulose<br>75 pph EVA, and<br>120 pph magnesium hydroxide                                           | 25                         | 271                                    |
| 9      | 100 pph NF03A starch, and<br>120 pph magnesium hydroxide                                                     | 14                         | 241                                    |
| 10     | 100 pph EVA, and -<br>120 pph magnesium hydroxide                                                            | 29                         | 410                                    |
| 11     | 100 pph PE, and<br>120 pph magnesium hydroxide                                                               | 30                         | 227                                    |
| 12     | 100 pph NF03 starch, and<br>150 pph magnesium hydroxide                                                      | 13                         | 238                                    |
| 13     | 100 pph NF03 starch, and<br>150 pph aluminum hydroxide                                                       | 13                         | 129                                    |
| 14     | 100 pph NF03 starch, and<br>150 pph hydrated magnesium carbonate and calcium and magnesium carbonate mixture | 12                         | 142                                    |
| 15     | 100 pph PLA-polyester 219F, and<br>150 pph magnesium hydroxide                                               | 14                         | 232                                    |
| 16     | 100 pph PLA-polyester 219F, and<br>150 pph aluminum hydroxide                                                | 13                         | 101                                    |
| 17     | 100 pph PLA-polyester 219F, and<br>150 pph calcium and hydrated magnesium carbonate                          | 13                         | 161                                    |
| 18     | 100 pph NF08 starch, and<br>40 pph aluminum hydroxide                                                        | 17                         | 289                                    |

The origins of the fire-retardant fillers used in samples 8 to 18 are as follows:

magnesium hydroxide and aluminum hydroxide are sold by the supplier Martinswerk under the references Magnifin H10 and OL 104 respectively; and

the mixture of hydrated magnesium carbonate and of calcium and magnesium carbonate is sold by the supplier Minelco under the reference Ultracarb U5.

On sight of the results of Table 4, samples in accordance with the invention present better fire-retardant properties since the heat of combustion of samples 8, 9, and 12 to 18 in accordance with the invention are much smaller than those of samples 10 and 11 for heat release peak values that are smaller or equivalent.

In order to show the advantages obtained in another particular embodiment of the present invention, and by way of example, two different biopolymers, namely 75 pph starch and 25 pph cellulose were mixed and molded in a press under the same conditions as specified above.

The sample obtained in that way presented tensile strength of 19 MPa and elongation at break of 70%.

Thus, mixing those two biopolymers advantageously presents mechanical properties that are well balanced, with ten-

## 6

sile strength being greater than that of sample 2 and elongation at break greater than that of sample 1.

Finally, to validate the use of compositions of the present invention in a cable application, compositions 1, 2, 5, and 5bis in Table 1 were extruded onto a metal conductor having a diameter of 1.03 mm to form a layer with a thickness of about 0.50 mm so as to obtain respective electric wires 1, 2, 5, and 5bis.

The extrusion profile for composition 1 extended from 145°C. to 200°C. at a pressure of 150 bar, that of composition 2 extended from 100°C. to 135°C. at a pressure of 135 bar, and that of compositions 5 and 5bis extended from 120°C. to 150°C. under a pressure of 190 bar, these extrusion profiles being well known to the person skilled in the art.

15 The extruded compositions were subjected to insulation testing. The insulation test in compliance with standard IEC 60502-1 includes immersing the electric wires in water for at least one hour before performing said test.

A direct current (DC) voltage lying in the range 80 volts 20 (V) to 500 V is then applied for a sufficient duration (in the range 1 min to 5 min), and then the resistance of the ring was measured. That makes it possible to determine the insulation constant.

The insulation constants (Ki) at 20°C. obtained for the 25 extruded compositions of electric wires 1, 2, 5, and 5bis are summarized in Table 5 below.

TABLE 5

| Extruded composition | Ki at 20°C. |
|----------------------|-------------|
| 1                    | 850         |
| 2                    | 5           |
| 5                    | 2.2         |
| 35 5bis              | 10.8        |

These values of Ki are advantageously greater than those recommended for certain materials, in particular for polyvinyl chloride.

40 Extruding said composition makes it possible to obtain layers of considerable thickness, of the order of at least 0.3 mm to 0.5 mm, unlike film coatings, thus making it possible to obtain good insulating properties. The greater the extruded thickness, the better the electrical insulation.

45 It is specified that the compositions in question are used in making insulating extruded materials and/or sheathing materials and/or cable-filler materials for power cables and/or telecommunications cables.

The composition may also include other additives, in particular antioxidants, UV stabilizing agents, plasticizing agents, pigmentation agents, and/or coloring agents.

Advantageously, plasticizing agents may be added to the composition in accordance with the present invention in order to improve the elongation at break of said composition.

55 55 By way of example, as a plasticizing agent, mention can be made of castor oil, crodamide, and triethyl citrate.

The present invention is not limited to the composition examples described above, and it bears more generally on all cables that can be envisaged on the basis of the general indications given in the description of the invention.

What is claimed is:

1. A power and/or telecommunications cable comprising: at least one component element made of a material extruded from an extrudable composition, wherein said extrudable composition is made from a biopolymer selected from the group consisting of polymers of cellulose ester, polymers of starch complexed with a bio-

degradable polyester, polymers of polyhydroxyalkanoate, and polymers of polylactic acid comprising a mixture of polylactic acid and of polyester, said polylactic acid polymers make up at least 40% by weight polylactic acid.

2. A power and/or telecommunications cable according to claim 1, wherein said extrudable composition also includes a synthetic polymer.

3. A power and/or telecommunications cable according to claim 2, wherein said synthetic polymer is selected from the group consisting of polyethylene, polypropylene, ethylene vinyl acetate copolymer, polyvinyl chloride, and polyester, and mixtures thereof.

4. A power and/or telecommunications cable according to claim 1, wherein said component element is selected from the group consisting of an insulating cover, a protective sheath, and a cable-filler material.

5. A power and/or telecommunications cable according to claim 1, wherein the polylactic acid polymers make up about 40% by weight polylactic acid and about 60% by weight polyester. 20

6. A power and/or telecommunications cable according to claim 1, wherein the cellulose ester polymers are selected from the group consisting of cellulose butyrate polymer, cellulose acetate polymer, and cellulose propionate polymer.

7. A power and/or telecommunications cable according to claim 1, wherein the polyhydroxyalkanoate polymer is a homopolymer or a copolymer of poly(3-hydroxybutyrate).

8. A power and/or telecommunications cable according to claim 1, wherein said extrudable composition further includes a fire-retardant filler.

9. A power and/or telecommunications cable according to claim 8, wherein the fire-retardant filler is selected from the group consisting of aluminum trihydroxide  $\text{Al(OH)}_3$ , magnesium dihydroxide  $\text{Mg(OH)}_2$ , a mixture of hydrated magnesium carbonate and calcium and magnesium carbonate, zinc borate, and/or cork powder.

10. A power and/or telecommunications cable according to claim 1, wherein the polylactic acid polymers make up no more than about 90% by weight polylactic acid.

\* \* \* \* \*